

# UNITED STATES PATENT OFFICE.

LYNDALL FORSE, OF YEOVIL, ENGLAND, ASSIGNOR OF ONE-THIRD TO SIDNEY THEODORE THRING AND ONE-THIRD TO REGINALD JOHN LUFTMAN, OF YEOVIL, ENGLAND.

## MANUFACTURE OF MOCHA LEATHER.

1,339,751.

Specification of Letters Patent. Patented May 11, 1920.

No Drawing.

Application filed December 29, 1916. Serial No. 139,579.

To all whom it may concern:

Be it known that I, LYNDALL FORSE, of "Silchester," Grove avenue, Yeovil, Somerset, England, subject of the King of Great Britain and Ireland, have invented certain new and useful Improvements in or Relating to the Manufacture of Mocha Leather, of which the following is a specification.

This invention relates to the manufacture of Mocha leather. The object of this invention is to provide an improved method of manufacture.

In the manufacture of Mocha leather as hitherto carried out the grain of the leather is removed by placing the skins in a vat or pit where they are allowed to soak and when the surface has been destroyed the skins are placed on a beam and the grain removed by a beam knife. According to this invention each skin is placed on a table or board and the granular surface destroyed by the application of any suitable agent which may be washed off when the grain has been affected to a sufficient extent, as is known to a trained and expert operator by the appearance of the skin, supplemented, if necessary, by an actual test on a small portion of the skin. For the purpose of carrying out this invention, an agent composed of caustic soda 12½%, caustic potash 12½% and water 75% may be employed, but I do not bind myself to the use of this agent. Any agent which will attack the skin has, to a certain extent, a similar action, but some reagents take an inconveniently long time to produce the required degree of disintegration of the granular surface, while the action of others is not thoroughly under control, so that the details of the process have to be varied according to the kind of skin under treatment, the nature of the reagent employed and the use the finished product is intended for, for instance, as to whether the prepared skin is to be dyed, or not. The agent may

be applied by a brush, sponge, spray or otherwise.

When the skin has been dried the surface is ground off by an emery or other grinding wheel.

In accordance with this method of manufacture only one surface of the skin is attacked, resulting in a saving in the texture and a plumper skin. The time and cost of manufacture is considerably reduced, and the loss due to skins being damaged in the pit process is avoided.

What I claim and desire to secure by Letters Patent is:—

1. The method of manufacture of Mocha leather characterized by applying on one side only of a skin a solution of an agent adapted to attack the skin, thereupon completely removing the whole granular surface of the skin, thereby producing a leather which is soft and velvety throughout.

2. The method of manufacture of Mocha leather characterized by applying on one side only of the skin a solution of an alkaline reagent adapted to attack the skin, thereupon completely removing the whole granular surface of the skin, thereby producing a leather which is soft and velvety throughout.

3. The method of manufacture of Mocha leather characterized by applying an agent composed of caustic soda 12½%, caustic potash 12½% and water 75% on one side of the skin only, thereupon completely removing the whole granular surface of the skin, thereby producing a leather which is soft and velvety throughout.

In witness whereof I have hereunto signed my name in the presence of two subscribing witnesses.

LYNDALL FORSE.

Witnesses:

FRANK E. SPERRING,  
MARGARET WELCH.